

June 22, 1937.

F. J. TONE

2,084,513

ABRASIVE ARTICLE

Original Filed Feb. 7, 1928



INVENTOR

Frank J. Tone  
by his attorney  
Byrne, Stithis, Arnolds, Banks

## UNITED STATES PATENT OFFICE

2,084,513

## ABRASIVE ARTICLE

Frank J. Tone, Niagara Falls, N. Y., assignor, by  
mesne assignments, to The Carborundum Com-  
pany, Niagara Falls, N. Y., a corporation of Del-  
aware

Continuation of application Serial No. 252,468,  
February 7, 1928. This application September  
26, 1930, Serial No. 484,545. Renewed October  
10, 1934

8 Claims. (Cl. 51—207)

The present invention relates to abrasive de-  
vices, and particularly to wheels, and pertains  
especially to abrasive wheels of such large size  
that they cannot be conveniently or economically  
5 molded and burned as an integral wheel, but is  
not limited to such particular application. The  
invention constitutes a continuation of my ap-  
plication Serial No. 252,468, filed February 7,  
1928.

10 More particularly the invention is especially  
applicable to the manufacture of pulp grinding  
wheels in connection with which it will be specif-  
ically described, but it is to be understood that  
it is not limited to such devices.

15 Pulp wheels are ordinarily several feet in di-  
ameter and of considerable width. They have  
commonly been cut from natural sandstone. More  
recently artificial abrasives have been used to  
some extent for this purpose. It is not practical  
20 to form a pulp wheel as an integral mass from  
an abrasive mix, due to the fact that the bond  
employed is generally a ceramic bond which  
must be fired to a high temperature to mature.  
It is extremely difficult to fire such a large mass  
25 and to secure the necessary heat penetration;  
moreover, such a mass in the green state cannot  
be conveniently handled without likelihood of  
damage, and in firing it is apt to slough away or  
warp. If other bonds are used in the abrasive  
30 mix, it is difficult to secure uniform curing  
throughout the entire mass.

Consequently, where artificial abrasives have  
been employed, the wheel has been formed of  
35 segments which are burned individually and as-  
sembled into the completed wheel. The general  
practice heretofore has been to provide a metal  
drum or cylinder to which the abrasive segments  
are secured and which forms a necessary part of  
40 the wheel assembly. Due to the fact, however,  
that metal cylinders and the abrasive segments  
have widely different coefficients of thermal ex-  
pansion, stresses are produced in such a wheel  
45 necessitating the use of some compensating ar-  
rangement to prevent breakage of the wheel over  
the temperature range to which the wheels are  
subjected to use. Ordinarily this temperature  
range is between -40° F. and 212° F. In such a  
50 wheel the metal drum is a very expensive part  
of the assembly. It costs several hundred dol-  
lars, at least, and considerably more if it is made  
of a material that will resist corrosion for pe-  
riods up to seven years, which is the length of  
55 time manufactured abrasive wheels last in pulp  
grinding operations.

55 The abrasive manufacturer assembles the seg-

ments on the metal drum, and the assembly is  
shipped to the user. The user operates the wheel  
until most of the abrasive has been worn off, when  
he returns the drum to the abrasive manufacturer  
to have the abrasive segments replaced. The  
metal drum, of course, adds materially to the  
shipping weight of the wheel as well as to the  
initial cost, and the freight cost of returning  
such a large metal cylinder to the abrasive manu-  
facturer is a further item of expense in the use  
5 of such wheels. In addition to this, the user of  
the wheels must have one or more spare wheels  
in stock at all times, so that operation of the mill  
will not be shut down during the time that a  
metal drum is in the hands of the abrasive manu-  
facturer for the replacement of the abrasive.  
10 This means that a considerable investment is un-  
productively tied up in the metal cylinders at  
15 all times.

According to the present invention, there is  
provided an abrasive wheel made of a plurality of  
20 preformed segments or members of abrasive ma-  
terial which are cemented together by a cement,  
the tensile strength of which is great enough  
to hold the segments together against the cen-  
trifugal and other forces incident to the opera-  
25 tion of grinding, whereby the use of a metal sup-  
porting drum is rendered unnecessary. The elim-  
ination of the metal drum in the wheel assem-  
bly effects a saving of from eight hundred to  
30 eighteen hundred dollars in the initial cost of  
a large pulp wheel, and a pulp wheel embodying  
the present invention will furnish the abrasive  
user with about one and one-half times as much  
35 abrasive for the same cost as a pulp wheel having  
abrasive segments on a metal drum; moreover,  
due to the elimination of the metal drum, the  
handling of the wheels is much easier.

The elimination of the metal supporting drum,  
however, introduces several serious problems into  
the successful use of the wheel, all of which are  
eliminated in the present invention. These  
wheels are shipped into territories and are used  
in places where the temperature not infrequent-  
ly gets as low as -40° F. In the operation of  
40 grinding pulp, the wheels are exposed to the  
action of water at about the boiling point. The  
wheel must be constructed so as to eliminate  
stresses or strains sufficient to produce any rup-  
ture thereof over this temperature range.

45 The material used for joining the segments  
must not only have a tensile strength great  
enough to hold the segments together against  
the centrifugal and other forces incident to the  
50 operation of grinding, but it also should have  
55

a modulus of elasticity such as to cause the joint to compress or to stretch readily when the abrasive segments expand or contract; moreover, its own coefficient of thermal expansion should be such with respect to its modulus of elasticity that any change in the size of the joint itself with an increase or decrease in temperature will not impose any undue strain on the wheel. According to the present invention, there is provided an abrasive wheel in which this relation of the joint material to the bonded abrasive material exists.

The invention may be described in connection with the accompanying drawing in which

Figure 1 is an elevation of a composite abrasive wheel embodying my invention;

Figure 2 is a section along the plane of line II-II of Figure 1;

Figure 3 is a plan view of the abrasive wheel;

Figure 4 is a vertical section showing the composite abrasive wheel with its mounting; and

Figure 5 is a plan view of the composite abrasive wheel containing a plurality of rings which are composed of different materials, the said rings having different abrasive properties and different physical properties in other respects.

The abrasive wheel shown in Figures 1 to 4 is made up of a number of segments 2 arranged in circumferentially extending rows 3, 4 and 5. The segments or blocks 2 are united by joints 30 designated 6, 7, 8 and 9. The end faces of the outer row of segments 3 and 5 are cut away to leave the projections 10 which are engaged by the end clamping plates 11, by means of which the wheel is mounted on a shaft 12. The wheel, as made by the abrasive wheel maker, is shown in Figures 1, 2 and 3, and the purchaser or user of the wheel mounts it as shown in Figure 4. It will be observed that the manner of mounting does not require the use of any internal cylinder 40 or other internal support, the two end plates providing the only means for supporting the wheel on the shaft. According to the preferred construction of the wheel, the segments in one row are staggered or offset with respect to the segments in the adjacent rows whereby the joints do not extend continuously transversely across the wheel.

The segments 2 are made of bonded abrasive grains. The bonding material used for bonding 50 the grains may be of any suitable kind, as for instance ceramic bonds, rubber, resins or the like. In the case of ceramic bonded segments, the blocks are molded and then fired in a kiln, after which the faces of the blocks are dressed to remove any loose material or protuberances from their faces.

The cement for uniting the segments and forming the joints should have a low modulus of elasticity with respect to that of the bonded abrasive, if it has a relatively high coefficient of thermal expansion. A material that has a relatively high modulus of elasticity should have, in general, a coefficient of expansion the same as, or only moderately higher than, that of the bonded abrasive. Where the wheel is used as a pulp wheel, the cementitious material forming the joints should retain sufficient strength after immersion in hot water for long periods of time to hold the blocks against the forces incident to the grinding operation.

I have found that synthetic resins possessing these properties are highly satisfactory for this purpose. Such synthetic resins should have incorporated therein some inert filling material, and the character of the joint can be varied by

varying the percent of inert filling material with respect to the amount of synthetic resin used.

As an example, one composition suitable for the purpose is as follows:

Composition:

|                                                   | Percent by weight | 5  |
|---------------------------------------------------|-------------------|----|
| Fused quartz 200 mesh and/or finer (inert filler) | 70                |    |
| "A" stage phenolic resin                          | 10                |    |
| Water                                             | 20                | 10 |

This material possesses the following properties:

|                                  |                                      |    |
|----------------------------------|--------------------------------------|----|
| Coefficient of thermal expansion | $3 \times 10^{-6}/^{\circ}\text{C.}$ | 15 |
| Modulus of elasticity            | $0.9 \times 10^6/\text{sq. in.}$     |    |

Another example of a synthetic resin is as follows:

Composition:

|                                                 | Percent by weight | 20 |
|-------------------------------------------------|-------------------|----|
| Inert filler fused quartz 200 mesh and/or finer | 84                |    |
| Glycerol-phthalic anhydrite resin               | 16                |    |

This mix is plasticized with 30 cc. of ethyl alcohol/100 gms. mix. 25

The cured material has the following characteristics:

|                          |                                        |    |
|--------------------------|----------------------------------------|----|
| Coefficient of expansion | $7.5 \times 10^{-6}/^{\circ}\text{C.}$ | 30 |
| Modulus of elasticity    | $1.0 \times 10^6/\text{sq. in.}$       |    |

A third example comprises:

|                                    | Percent by weight |    |
|------------------------------------|-------------------|----|
| Inert filler 240 mesh and/or finer | 86                |    |
| "A" stage phenolic resin           | 14                | 35 |

This mixture has the following physical properties:

|                          |                                      |    |
|--------------------------|--------------------------------------|----|
| Coefficient of expansion | $9 \times 10^{-6}/^{\circ}\text{C.}$ |    |
| Modulus of elasticity    | $2.7 \times 10^6/\text{sq. in.}$     | 40 |

Still another example of a suitable material comprises:

|                                       | Percent by weight |    |
|---------------------------------------|-------------------|----|
| Fused quartz 200 mesh and/or finer    | 68.3              |    |
| "A" stage phenolic condensation resin | 19.5              | 45 |
| Water                                 | 12.2              |    |

This material has the following physical characteristics:

|                                  |                                        |    |
|----------------------------------|----------------------------------------|----|
| Modulus of elasticity            | $1.8 \times 10^6/\text{sq. in.}$       | 50 |
| Coefficient of thermal expansion | $7.6 \times 10^{-6}/^{\circ}\text{C.}$ |    |

Theoretically, in the above mixes, it would be desirable to have the moduli of elasticity reversed in order; however, a modulus of elasticity of  $2.7 \times 10^6$  is low enough for a cement having a coefficient of expansion of  $9 \times 10^{-6}$ , and consequently it is immaterial that those cements with lower coefficients of expansion have lower moduli of elasticity. 60

I have also found that the characteristics of hard rubber can be modified to adapt it to the cementing of abrasive segments in a wheel of this nature, or for the cementing of abrasive articles having different coefficients of thermal expansion and elasticity. A typical example is:

|                                                         | Parts by weight |      |
|---------------------------------------------------------|-----------------|------|
| Rubber                                                  | 10.0            |      |
| Sulphur                                                 | 2.5             |      |
| Silicon carbide at a fineness of approximately 500 mesh | 70              | 90.0 |

When this mix is cured to the extent required by the percentage of sulphur given above, it is satisfactory as a joint material for a medium

grade wheel having a specific type of bond and a specific type of abrasive, but it would not necessarily be applicable to a wheel of a different grade of abrasive, or having a different bond or using a different abrasive material. This composition, when cured, has the following properties:

Tensile strength 2,000 lbs. per sq. in.  
Coefficient of thermal expansion  $20 \times 10^{-6}/^{\circ}\text{C}$ .  
Modulus of elasticity  $1.5 \times 10^8 \text{#/sq. in.}$

In order to provide cement suitable for other materials, it is only necessary to vary the composition as given above, in accordance with the following general trends until the desired properties are obtained.

The inert filler, being of relatively low coefficient of thermal expansion with respect to the rubber sulphur compound, serves to reduce the coefficient of thermal expansion of the joint material in proportion to the amount present. Consequently, by increasing the amount of inert filler from the percentage given above, the coefficient of thermal expansion of the joint material is lowered while the modulus of elasticity is slightly increased. Generally stated, the modulus of elasticity of the joint material increases in proportion to the degree of vulcanization of the rubber and in proportion to the amount of inert filler present.

Other materials can be used in place of silicon carbide, as the inert filler. For instance, alumina or quartz, as noted above in the synthetic resin cements, can be employed.

The inert filler preferably has a coefficient of thermal expansion not substantially greater than that of fused quartz, which is about  $.5 \times 10^{-6}$  per degree centigrade.

The following specific methods of joining members to make a unitary structure are given where rubber is employed by way of illustration and are not intended to limit the invention to the specific materials or manipulative details disclosed, nor are they intended to limit the process to the specific steps or sequence of steps.

The abrasive surfaces that are to be joined are first primed with the rubber compound softened with a volatile softener, such as benzol. The ratio of benzol to rubber compound may be varied as required, but it has been found that two parts of benzol and one part of the rubber compound form a priming material that may be applied easily by brushing and leaves a satisfactory coating of rubber compound on the abrasive surface after the solvent has evaporated. If a thicker coating of rubber compound than that produced by one application, either by brushing or by spraying, is desired, additional coats of the solvent-softener compound may be applied. Sufficient time should elapse between coatings to permit the solvent to evaporate completely before a subsequent coat is applied.

The blocks or rings of bonded abrasive material are then positioned with a sheet of the joint material, of the desired thickness and of the area of the block or ring, between them. Pressure is applied to force the joint material into intimate contact with the surfaces it lies between, and heat is applied to cure the joint material.

Figure 5 illustrates a two-part abrasive wheel in which the two parts 13 and 14 have different grinding characteristics. For example, the ring 13 may be intended for rapid cutting, this ring being made from a vitrified disk with a siliceous bond of very low coefficient of expansion used to

hold together coarse grain consisting of fused alumina. The ring 14 may be made of finer grains of silicon carbide bonded with rubber or phenol condensation product resin. The coefficient of expansion of a rubber bond is in general greater than that of a highly siliceous bond. The two rings are cured separately according to the methods suitable for the two types of bond respectively. The two rings are then united by means of a cement whose coefficient of expansion and resiliency are such that the abrasive materials in the respective rings will not suffer undue stress under the extreme temperature and speed conditions to which they are subjected.

The composite wheel structure provided by the present invention comprises, generally stated, a plurality of segments which are set in and held together by a web or skeleton of cementitious material which holds the blocks together against the centrifugal and other stresses incident to operation, and the thermal expansion of which and modulus of elasticity of which are adjusted in accordance with the abrasive employed whereby the structure is free of any strains over the temperature range to which it is subjected under normal conditions.

The invention, therefore, provides a practical way in which a substantially solid body of abrasive material can be employed without metal supporting drums. Pulp wheels made in accordance with the present invention have been satisfactorily employed over extended periods of time. The initial cost of such wheels has been proven much less than the cost of wheels employing metal reinforcing drums. The joint material is resistant to the action of hot water, so that the rate of disintegration of the joints is not excessive in proportion to the rate of disintegration of the abrasive blocks themselves.

The cements above described being somewhat elastic, apparently allow a certain amount of yield in the structure, whereby the blocks can adjust themselves under the strains set up upon operation of the wheel; moreover, joints of the materials disclosed herein have a tensile strength at least 200#/sq. inch after continuous immersion in boiling water for periods of four weeks or more.

While I have described my invention with particular reference to pulp wheels, it will be understood that the invention is not so limited but may be used in the manufacture of other composite abrasive articles.

I claim:

1. An abrasive wheel, comprising a plurality of preformed shapes of bonded abrasive material and having cementitious joints between the abrasive shapes composed of a phenolic condensation resin binder together with at least 70% by weight of the total of fused quartz ground 200 mesh and finer, said cementitious joint material being characterized by a coefficient of thermal expansion approximately that of the bonded abrasive and a modulus of elasticity in the order of about  $1 \times 10^8$  to  $3 \times 10^8$  pounds per square inch, and forming joints with the abrasive shapes having a tensile strength of at least 200 pounds per square inch after continuous immersion in boiling water for four weeks.

2. An abrasive wheel, comprising a plurality of preformed shapes of bonded abrasive material and having cementitious joints between the abrasive shapes composed of a synthetic resin binder together with at least 70% by weight of a finely divided inert filler having a relatively low

- coefficient of thermal expansion, said cementitious joint material being characterized by a low modulus of elasticity with respect to that of the bonded abrasive.
3. An abrasive wheel, comprising a plurality of preformed shapes of bonded abrasive material and having cementitious joints between the abrasive shapes composed of a synthetic resin binder and a finely divided inert filler, said cementitious joint material being characterized by a coefficient of thermal expansion of the same order as that of the bonded abrasive and a modulus of elasticity lower than that of the bonded abrasive, and forming joints with the abrasive shapes having a tensile strength of at least 200 pounds per square inch after continuous immersion in boiling water for four weeks.
4. An abrasive wheel, comprising a plurality of preformed shapes of bonded abrasive material and having cementitious joints between the abrasive shapes composed of a hard rubber binder together with a finely divided inert filler having a thermal expansion lower than that of the hard rubber.
5. An abrasive wheel, comprising a plurality of preformed shapes of bonded abrasive material and having cementitious joints between the abrasive shapes composed of a hard rubber binder together with a finely divided inert filler having a thermal expansion lower than that of the hard rubber, the rubber and filler being so proportioned that the cementitious joint material has a coefficient of thermal expansion approximating that of the bonded abrasive and a modulus of elasticity lower than that of the bonded abrasive,
- and forming joints with the abrasive shapes having a tensile strength of at least 200 pounds per square inch after continuous immersion in boiling water for four weeks.
6. An abrasive wheel comprising a plurality of preformed shapes of bonded abrasive material and having cementitious joints between the abrasive shapes composed of a synthetic resin binder together with a finely divided inert filler having a coefficient of thermal expansion not substantially greater than that of fused quartz, the binder and filler being so proportioned that the cementitious joint material has a coefficient of expansion approximating that of the bonded abrasive and a modulus of elasticity lower than that of the bonded abrasive.
7. An abrasive wheel comprising a plurality of preformed shapes of bonded abrasive material and having cementitious joints between the abrasive shapes composed of a phenolic condensation resin binder together with at least about 68% by weight of the total of finely divided fused quartz.
8. An abrasive wheel comprising a plurality of preformed shapes of bonded abrasive material and having cementitious joints between the abrasive shapes composed of a synthetic resin binder together with an inert filler having a coefficient of thermal expansion not substantially greater than that of fused quartz, the binder and filler being so proportioned that the cementitious joint material has a coefficient of expansion approximating that of the bonded abrasive and a modulus of elasticity lower than that of the bonded abrasive.

FRANK J. TONE. 35